

No. 800,223.

PATENTED SEPT. 26, 1905.

M. LEITCH.  
TREATING TIN SCRAP.  
APPLICATION FILED OCT. 19, 1904.



Fig. 3.



Witnesses  
Charles A. Peard  
L. Vreeland

Inventor  
Meredith Leitch  
By his Attorneys  
Barrett Maxwell Mitchell

# UNITED STATES PATENT OFFICE.

MEREDITH LEITCH, OF BROOKLYN, NEW YORK.

## TREATING TIN-SCRAP.

No. 800,223.

Specification of Letters Patent.

Patented Sept. 26, 1905.

Application filed October 19, 1904. Serial No. 229,071.

*To all whom it may concern:*

Be it known that I, MEREDITH LEITCH, a citizen of the United States, residing at Brooklyn, Kings county, New York, have invented 5 certain new and useful Improvements in Treating Tin-Scrap, of which the following is a full, clear, and exact description.

My invention relates to improvements in treating tin-scrap, by which I mean tin cuttings, old tin cans, and the like, so as to recover the tin from the same in an economical and efficient manner.

Heretofore tin-scrap has been subjected to electrolytic action in a suitable electrolyte, 15 such as caustic soda, and the tin in that way removed from the cans and deposited on suitable cathodes. It has been the practice to subject tin-scrap made up of trimmings to the action of the electrolyte without any previous treatment. In the case of tin cans and the like it has been the practice to puncture or cut out the cans, so that the electrolyte can circulate through them freely, and in some cases to remove the labels by washing. Both 20 25 30 35 40 45 50 55 60 65 70 75 80 85 90 95 100 105 110 of these steps in the preparation of the cans for the electrolytic bath are slow and expensive and, while entailing extra expense, are quite unsatisfactory in their results. The principal difficulty is that even after the cans are washed as thoroughly as they can be by any commercial washing process some paste, oil, grease, and vegetable matter adheres to them, while in the case of trimmings the palm-oil which is applied to the tin as it leaves the tinning-bath adheres. These substances adhering to the tin are known in the art as "filth," which is the bane of electrolytic processes, since it interferes with the action of the electrolyte. When caustic soda is used, the oil and grease combine with it to make soap, while the vegetable matter is attacked by it and causes it to deteriorate so as to soon be unsuitable for use. The problem therefore is how to remove the filth or change it into some form which will not interfere with the electrolyte and to do this economically and satisfactorily without destroying the tin which it is desired to save. I have discovered a process by which these results can be attained, which, broadly stated, consists in converting the filth into a substance inert, so far as the electrolyte is concerned, and doing this without destroying the tin.

Specifically stated, the process consists in 55 driving off the volatile portions of the filth

and in carbonizing the remainder by subjecting it to a carbonizing temperature in a deoxidized atmosphere.

A further improvement consists in agitating the cans in such a manner as to dislodge 60 much, if not all, of the carbonized material, and thereby separate it from the scrap before the scrap is subjected to the electrolyte. The treatment of the tin cans in the absence of oxygen preserves the tin, which otherwise would 65 be lost.

The process, in addition to the advantageous results above specified, also has the advantage in that in some forms of apparatus for carrying out my improvements the solder 70 can simultaneously be practically all removed from the tin cans so that it does not interfere with the detinning and is not present to lower the grade of iron of castings made from scrap after the detinning process is completed. 75 Furthermore, the solder itself which is removed is valuable and is thereby separated so that it also can be saved. The solder collected more than pays for the cost of carrying out the step which constitutes my present 80 improvement. My invention, however, is not necessarily allied to desoldering, since it can be carried out by mechanism which does not desolder. When it is carried out in a desoldering mechanism, however, it has the advantage of not only converting the filth into 85 an inert substance, but also the advantage of opening up the cans by separating the parts thereof so that the electrolyte can circulate freely through the scrap. 90

The following is a description of my invention, reference being had to the accompanying drawings, in which—

Figure 1 is a longitudinal section of the preferred form of apparatus adapted to be 95 used in carrying out my invention. Fig. 2 is a plan view of the same. Fig. 3 is a diagram.

Referring more particularly to the drawings, the apparatus to the left represents a centrifugal carbonizing and desoldering furnace, and the apparatus to the right represents a detinning-bath. In the furnace, A represents an inclosing wall provided with a door B, through which material can be removed from below. Within the chamber 100 formed by the wall A is a revolving basket or centrifugal separator D, preferably of steel, mounted upon the shaft E, which shaft is supported in bearings F F' and driven by the pulley G. This basket D is provided with 105 110

elongated perforations  $d$  in its sides for the purpose hereinafter described. The bearings  $F F'$  are of any well-known type suitable for use in connection with a heated shaft. Within the basket D extends a hopper H, preferably conical in form, as shown. This hopper forms a cover for the chamber formed by the wall A, being supported at the upper end of said wall, so as to seal the upper part of the chamber. The hopper is provided with spiral ribs I, which coat with teeth J on the revolving sleeve surrounding the shaft E in such way as to assist in forcing the material within the hopper downward into the basket D. The upper part of the chamber formed by the wall A and the hopper H is provided with an outlet K, the lower end of which dips into the tank L so as to be sealed by the electrolyte therein. The upper edge of the basket D is provided with a horizontal flange D', which extends over a horizontal flange D'', carried by the wall A, so as to substantially prevent matter rising above the edge of the basket from passing between the upright wall of the basket and the wall A. The pipe M extends through the wall A and into the basket D, where it is provided with orifices  $m$ . Through this pipe is supplied a mixture of gas and air by pipes N and O, respectively, said pipes being provided with stop-cocks  $n$  and  $o$  for controlling the supply of gas and air in such a way that the proportions shall be those necessary for the burning of the gas within the furnace without the leaving of any free oxygen.

At any convenient point or points on the circumference of the furnace I provide a feeding and disintegrating mechanism which assists in causing the cans or other matter within the basket D to be fed upward along its sides, so as to be discharged through the discharge-opening K, and also tends to knock the cans into pieces and to jar off carbonized material therefrom. This consists of a series of toothed disks P, mounted on a shaft Q, journaled at R and R' and inclosed by the covering S. The teeth upon these disks protrude through the elongated orifices  $d$  in the basket D, so that rotation of the basket produces rotation of the disks. If the shaft Q is exactly vertical, the only action of these disks is to hit the cans as they engage with the teeth, and thus jar them so as to cause the parts to separate and to remove the solder and more or less of the carbonized material thereon. In practice, however, the shaft Q is inclined slightly, in the direction opposite to the direction of rotation of the basket D, from which it results that the blows which the scrap within the basket D receive are in an upward direction and cause the scrap to move slowly upward along the sides of the basket D until discharged through the opening K. The angle of inclination of the shaft Q is preferably so slight that it cannot be shown in the drawings.

The disks B are, in effect, geared with the basket D and are rotated thereby on account of that engagement.

Fig. 3 shows the relation of the axis of the shaft Q to the axis of the shaft E, as would be seen in looking from the periphery at the left toward the center of the machine. The size of the angle is greatly exaggerated. In this figure, Q represents the axis of the shaft Q, and E represents the axis of the shaft E with its inclination exaggerated. The arrow represents the direction of rotation of the basket A in the apparatus of Figs. 1 and 2.

The tank L is of iron and forms the anode of the battery T, the cathode being the iron plates U, suspended from the bus-bar V. The liquid in this instance is caustic soda. The cans falling to the bottom of the tank are thus electrically connected to the anode and are acted upon electrolytically, the tin being deposited on the cathode U. I have not shown any means for distributing the cans in the tank L or removing them therefrom, since any proper means known to the art can be used for that purpose.

In carrying out my method with the apparatus above described I first feed the cans into the hopper H, meanwhile revolving the basket D by means of power applied to the pulley G, the gas and air mixture being supplied and ignited, so as to raise the temperature within the furnace to that required for carbonizing, and preferably to that required for melting the solder in the cans. The revolution of the basket, together with the sleeve connected thereto bearing the pins J, feeds the cans in the hopper downward into the basket D, where they are subjected to the action of heat and centrifugal force, with the result that as soon as the solder is melted it is thrown off by centrifugal force through the perforations  $d$  in the sides of the basket D, the sharp blows which the cans receive from the disks P aiding in the dislodgment of the solder and carbonized matter and also the disintegration of the cans. The solder is discharged by centrifugal force through the openings  $d$ , and the carbonized matter which has been dislodged also sifts through those openings and falls beneath the basket D, from which both solder and carbonized material are removed as necessary through the door B. The cans which are fed into the hopper H being pressed downward, together with the feeding-disks P, cause the desoldered cans, which are in the basket D, to move upward until they pass above the flange D', at which time the centrifugal force throws them outward to the exit K, provided for that purpose, by which they are conducted into the tank L. As above stated, the liquid in the tank L acts to prevent the egress of the products of combustion through the discharge-opening K, so that they can find exit only through the opening in the hopper H and in passing out through

this opening constitute a gas seal therefor and prevent the ingress of air at that point. The atmosphere within the furnace is therefore entirely deoxidized, and no oxidation of the material treated takes place within the furnace. The carbonaceous matters are thoroughly carbonized and the solder is removed. The tin coating is subsequently removed by the detinning-bath, being left intact by the action within the furnace. The cans are disintegrated and much of the carbonized matter shaken off, so that the cans are in condition to be subjected to the detinning-bath.

My invention is valuable not only when caustic-soda or other alkali process is used in detinning, but also when an acid process or the like is used, since it removes matter which would otherwise interfere with the desired result.

In the treatment of tin-scrap matter made up of trimmings by my process the volatile portion of the palm-oil which is ordinarily applied to the tin in its manufacture is driven off and the remaining carbonaceous matter carbonized, so that my improvement constitutes a marked advantage in the process of recovering tin from scrap of that kind, as well as from old cans and the like.

In case it is not desirable to detin the cans immediately after their discharge from the carbonizing-furnace the tank L can be filled with water, which acts to seal the discharge K. The cans may then be removed as desired and subjected to the detinning-bath at such time or place as may be convenient.

The mechanical features of the furnace shown and described herein are claimed in my copending application, Serial No. 232,420, filed November 12, 1904.

What I claim is—

1. In the treatment of tin-scrap for the recovery of tin by a detinning-bath the improvement which consists in converting the filth adhering to said scrap into a form not detrimental to the bath without removing the coating of tin and keeping the medium surrounding the scrap while being thus treated inert relatively to the tin thereon.

2. In the treatment of tin-scrap for the recovery of tin by a detinning-bath the improvement which consists in volatilizing the volatile portions of the filth and carbonizing the carbonaceous matter of the filth and meanwhile keeping the medium surrounding the scrap deoxidized and at a temperature sufficiently high to carbonize the carbonaceous

matters but not high enough to remove the coating of tin from the scrap.

3. In the treatment of tin scrap for the recovery of tin by a detinning-bath the improvement which consists in volatilizing the volatile portions of the filth and carbonizing the carbonaceous matters of the filth in a deoxidized atmosphere heated sufficiently to carbonize the carbonaceous matters but not to remove the tin coating from the scrap and jarring said scrap so as to remove the carbonized matter therefrom.

4. In the process of treating tin-scrap comprising old tin cans for the recovery of tin by a detinning-bath the improvement which consists in volatilizing the volatile portions of the filth and carbonizing the carbonaceous matter of the filth in a heated deoxidized atmosphere without removing the tin coating and subjecting the cans while in said heated atmosphere to mechanical blows and thereby disintegrating them.

5. In the process of treating tin-scrap consisting of old tin cans, the improvement which consists in subjecting the same to heat in a deoxidized atmosphere and subjecting the cans thus heated to mechanical blows.

6. In the process of treating tin-scrap consisting of old cans, the improvement which consists in subjecting the same to heat in a deoxidized atmosphere and periodically striking the cans thus heated and thereby disintegrating them and impelling them in an onward direction.

7. In the process of treating tin-scrap consisting of old cans, the improvement which consists in subjecting the same to heat in a deoxidized atmosphere and striking the cans thus heated with blows in an obliquely onward direction and impelling them onward by such blows.

8. In the process of treating tin-scrap consisting of old cans, the improvement which consists in subjecting the same to heat in a deoxidized atmosphere and simultaneously subjecting them to centrifugal force and striking them with blows in an obliquely onward direction thereby causing them to move onward and to become disintegrated.

Signed at New York city, New York, this 18th day of October, 1904.

MEREDITH LEITCH.

Witnesses:

H. M. SKINNER,  
L. VREELAND.